

Mar. 3, 1925.

1,528,099

C. F. CROMMETT

METHOD OF DECOMPOSING HYDROCARBONS

Original Filed May 24, 1922



Inventor.  
Charles F. Crommett  
by Heard Smith & Tenant.  
Atlys.

Patented Mar. 3, 1925.

## UNITED STATES PATENT OFFICE.

CHARLES F. CROMMETT, OF CHELSEA, MASSACHUSETTS, ASSIGNOR OF ONE-THIRD TO  
WILFORD J. HAWKINS, OF NEW YORK, N. Y., AND ONE-THIRD TO LOUIS N.  
WHEELOCK, OF BOSTON, MASSACHUSETTS.

## METHOD OF DECOMPOSING HYDROCARBONS.

Application filed May 24, 1922, Serial No. 563,385. Renewed January 28, 1925.

*To all whom it may concern:*

Be it known that I, CHARLES F. CROMMETT, a citizen of the United States, and resident of Chelsea, county of Suffolk, State of Massachusetts, have invented an Improvement in Methods of Decomposing Hydrocarbons, of which the following description, in connection with the accompanying drawing, is a specification, like characters on the drawing representing like parts.

This invention relates to a method of treating hydrocarbons or hydrocarbon compounds for the purpose of separating them into their constituent elements thereby to form carbon black and gases, or in some cases to form carbides and gases.

There are two methods now commonly employed for producing carbon black from hydrocarbons. One method involves burning the hydrocarbon with an insufficient amount of air thus resulting in the deposit of carbon black, and the other method involves subjecting the hydrocarbons to a very high heat (1300° C. to 1700° C.).

The first, or "limited combustion" method has the disadvantage that it is relatively inefficient as only a small percentage of the carbon in the hydrocarbon can be recovered as carbon black.

The second, or "high temperature" method also has the disadvantage that it is difficult to find suitable materials which will withstand the high temperatures required in carrying out this method and yet afford a practical means for withdrawing the carbon black when produced.

Furthermore in carrying out this "high temperature" process it has been found necessary to maintain the high temperature for a considerable period of time before the hydrocarbon is broken up into its constituent elements, and this relatively long period of high heat is destructive to the apparatus which is usually used.

An object of my present invention is to provide an improved method for decomposing hydrocarbon by the application of heat by which the desired end can be accomplished more rapidly than in prior methods and at a considerably less temperature than is required in the "high temperature" process.

Authorities state that when acetylene

(which is a hydrocarbon) is heated in the presence of a suitable catalyzing agent the temperature of dissociation of the constituents of the acetylene is considerably less than that which is required if the re-action is carried out without the presence of the catalyst.

In practising my invention I make use of this principle by heating the hydrocarbon compound in the presence of a catalyzing agent. I have found from experiment that it is advantageous to give the catalyzing agent a fluctuating temperature and my invention, therefore, involves passing the hydrocarbon compound over a heated catalyzer which has a fluctuating temperature.

For the purpose of giving a better understanding of the invention I have illustrated in the drawings more or less diagrammatically an apparatus which may be used for this purpose.

This apparatus consists of a passage or chamber 1 having an inlet 2 for the hydrocarbons and an outlet 3. Said passage is adapted to be heated in some suitable way as by means of a heater 4. The passage contains a catalyzing agent over which the hydrocarbon passes and in the illustration this catalyzing agent is in the form of a lining 5 for the chamber. 6 indicates a scraper movable longitudinally of the chamber and which may be used for scraping the carbon black from the walls of the passage, as it is deposited thereon, said carbon black being delivered into a collecting chamber 7 through a passage 8.

When the hydrocarbon is heated in the presence of the catalyzer, as is the case where it is heated in the passage 1 lined with a catalyzing agent, the dissociation of the hydrogen and carbon will take place at a much lower temperature than if the catalyzer was not present and will also take place at a more rapid rate, because of the presence of the catalyzer.

As stated above the catalyzer may be made of various metals which will have the desired catalyzing effect and the temperature which it is necessary to employ as well as the length of time it is necessary to subject the hydrocarbon to this critical temperature depends somewhat on the character of the catalyzer.

For instance, by using metallic palladium as the catalyzing agent and by heating the chamber or passage 1 to a temperature of between 700° C. and 750° C., I have obtained a yield of carbon black at the rate of about 18 lbs. per 1000 cubic feet of hydrocarbon in the form of methane.

Metallic nickel as a catalyst also gives excellent results but requires a slightly higher temperature than palladium, and as stated above good results can be obtained by using catalyzing agents of cobalt, magnesium, manganese, silicon, copper, etc.

In carrying out this method it is desirable to eliminate entirely from the hydrocarbon before heated in the presence of the catalyst any moisture or other oxygen-producing constituent, because if the hydrocarbon contains such a constituent, the latter becomes decomposed by the heat thus producing free oxygen which will unite with some of the carbon and will consequently decrease the production of carbon black.

The dissociation of the hydrogen and carbon is an endothermic operation, that is one which absorbs heat, and I find by experiment that the temperature in the chamber 1 varies somewhat notwithstanding the application of constant heat thereto, this varying temperature being due to the varying degree of absorption of heat by the dissociation of the gases. The action of the catalyst is augmented when its temperature fluctuates and my invention contemplates causing a fluctuation of the temperature of the catalyst from outside sources if it is found desirable to do so to stimulate the catalyzing effect. Such fluctuation can be produced by

providing means for electrically heating the catalyst periodically or by using any other means for thus periodically heating the catalyst in addition to the heat which is produced from the heater 4.

My invention, therefore, contemplates not only heating the hydrocarbon in the presence of the catalyst but also contemplates doing this with a catalyst having a fluctuating temperature, however such fluctuation may be secured.

In carrying out the process the carbon will be deposited on the walls of the passage 1 as dissociation takes place and the hydrogen or other gas is discharged through the discharge pipe 3 and may be used for any purpose, such for instance as providing heat which can be used in carrying out the process or operate a heat engine or performing any other useful work.

I claim:

1. The method of forming carbon black which consists in dehydrating a hydrocarbon mixture and then passing it through a heated passage containing a catalyzing agent which stimulates the dissociation of the carbon and hydrogen.

2. The method of decomposing a hydrocarbon compound, which consists in passing the compound over a heated catalyst having a fluctuating temperature.

3. The method of decomposing hydrocarbon which consists in heating said hydrocarbon in the presence of a catalyzing agent having a fluctuating temperature.

In testimony whereof, I have signed my name to this specification.

CHARLES F. CROMMETT.